

## UNITED STATES PATENT OFFICE

2,062,335

## GLASS METAL SEAL

Howard Scott, Wilkinsburg, Pa., assignor to Westinghouse Electric & Manufacturing Company, a corporation of Pennsylvania

No Drawing. Application July 5, 1929,  
Serial No. 376,291

14 Claims. (Cl. 176—36)

My invention relates to alloys and particularly to alloys of metals in the iron group of the periodic table.

One object of my invention is to provide an alloy having a predetermined coefficient of expansion over a temperature range from substantially room temperature to the annealing temperature of certain glasses, particularly boro-silicate glass and ordinary lead glass.

10 Another object of my invention is to provide an alloy having a smaller coefficient of expansion than the nickel-steel alloys.

Another object of my invention is to provide an alloy adapted to form a vacuum-tight seal 15 through boro-silicate glass.

Another object of my invention is to provide an alloy adapted to form a vacuum-tight seal through lead glass.

Another object of my invention is to provide an improved method of sealing electrical conductors 20 through glass.

A further object of my invention is to provide a method for producing a vacuum-tight seal of electrical conductors, having only a limited range 25 of expansivity substantially equal to that of ordinary glasses, through the latter without causing breakage of the seals in cooling to room temperature.

Other objects of my invention will become apparent on reading the following specification.

30 In connection with the manufacture of vacuum-tight electrical-discharge devices in glass containers, the problem arises of making vacuum-tight seals of metals through the glass walls. In forming such seals, a small hole is melted in the glass wall of the container; the metal lead is inserted and the molten glass squeezed around the lead and fused thoroughly in contact therewith. In order that the resulting seal shall not crack 40 or leak after it has cooled, it is necessary that the metal and the glass shall have substantially the same expansivity with temperature over the range from the annealing temperature of glass down to room temperature; and preferably that the metal be one which the glass will "wet". Platinum metal has the proper expansivity, when used in combination with ordinary lead glass, and the first successful seals through glass were made with platinum leads.

45 However, for certain purposes, it is desirable to use higher-melting glass than the ordinary lead glass just referred to; and hence, the use of boro-silicate glass in electrical apparatus has become fairly common. The boro-silicate glass, 50 however, has a materially lower coefficient of ex-

pansion than lead glass and, consequently, platinum seals could not be used in it. However, tungsten and molybdenum were found to have coefficients of expansion of the right order of magnitude and to form vacuum-tight seals with 5 boro-silicate glass. Such seals are, however, rather expensive and not entirely satisfactory.

Platinum, likewise, is an extremely expensive metal and, consequently, composite conductors having cores of nickel-steel covered by thin jackets of copper were developed, and thus cheaper, but equally satisfactory, seals through ordinary lead glass were obtained. The coefficient of expansion of copper is higher than that of lead glass; and, since the jacket of copper is relatively 10 thin, the nickel-steel alloy employed is one which has a coefficient of expansion nearly equal to that of lead glass. Copper is a metal which lead glass "wets" readily; and the expansivity of nickel-steel is slightly less than that of glass over the 15 range of approximately 400° C. between the temperature at which strains readily relieve themselves in lead glass and room temperature.

However, when the attempt was made to find 20 nickel-steels of the low expansivity corresponding to that of boro-silicate glass, it was found that, while this low expansivity existed up to a certain critical temperature, this temperature, herein called the inflection temperature, was considerably lower than that of the nickel-steel 25 alloys suitable for lead glass; and that, consequently, there was a range of temperature just below the proper annealing temperature of the glass in which the expansivity was so great that 30 vacuum-tight seals could not be produced.

In accordance with the present invention, I 35 have discovered that, by substituting cobalt for a certain part of the nickel in the nickel-steels previously employed, alloys result having sufficiently low coefficients of expansion throughout 40 the entire range below the necessary annealing temperature of boro-silicate glass; that such alloys are "wet" by the boro-silicate glass; and that the combination produces satisfactory vacuum-tight seals. Furthermore, I find that, by 45 employing certain other nickel-cobalt-iron alloys, and even certain nickel-iron alloys, seals may be made through ordinary lead glass; and this without the necessity for copper-jacketing the alloy.

50 In accordance with the foregoing principles, I have found that substitution of cobalt for nickel in nickel-iron alloys results in a decrease of expansivity of approximately  $0.5 \times 10^{-6}$  cm. per cm. per degree centigrade for each percent 55

of cobalt thus substituted. Ordinary lead glass has an expansivity of approximately  $9 \times 10^{-6}$  cm. per cm. per degree C. while boro-silicate glasses have expansivities between 3.0 and  $7.0 \times 10^{-6}$  cm. 5 per cm. per degree C. In accordance with the foregoing principles, I have found that alloys containing from 28% to 34% nickel, from 5 to 20% cobalt and from 0 to 1% manganese, the remainder of the alloy being iron, maintain an 10 expansivity over the temperature range up to the annealing temperature of boro-silicate glass, that is to say, up to about 400° C., which is a sufficiently near approximation to that of the glass to ensure a successful vacuum-tight seal. 15 In particular, I have found that an alloy comprising 32% nickel, 16% cobalt, 0.8% manganese, carbon up to 0.10% and the remainder iron, may be sealed successfully through boro-silicate glass having a coefficient of expansion 20 of substantially  $6.2 \times 10^{-6}$  cm. per cm. per degree C. As examples of such boro-silicate glasses, the following may be given:

1. 72.4%  $\text{SiO}_2$ ; 9.8%  $\text{Na}_2\text{O}$ ; 10.2%  $\text{B}_2\text{O}_3$ ; 5.1%  $\text{Al}_2\text{O}_3$ ; 1.8%  $\text{PbO}$ .  
 2. 67.0%  $\text{SiO}_2$ ; 6.4%  $\text{Na}_2\text{O}$ ; 19.0%  $\text{B}_2\text{O}_3$ ; 1.2%  $\text{Al}_2\text{O}_3$ ; 4.8%  $\text{Sb}_2\text{O}_3$ .  
 3. 73.8%  $\text{SiO}_2$ ; 18.7%  $\text{B}_2\text{O}_3$ ; 5.2%  $\text{PbO}$ ; 1.0%  $\text{Al}_2\text{O}_3$ ; 0.5%  $\text{As}_2\text{O}_3$ .

I have found that successful seals result 30 from the employment of alloys within the ranges of the composition heretofore described in conjunction with either of the aforesaid boro-silicate glasses.

I have further found that a successful seal 35 may be made between boro-silicate glass having an effective expansivity between 6.0 and  $6.5 \times 10^{-6}$  cm. per cm. per degree C. and an alloy containing substantially 27% nickel, 22% cobalt, 0.5% manganese and the remainder iron. 40 Likewise, I have found that alloys containing from 23% to 28% nickel, 17% to 23% cobalt, 0 to 0.5% manganese and 0 to 0.3% carbon may be sealed successfully in boro-silicate glasses 45 having effective expansivities between 3.0 and  $5.5 \times 10^{-6}$  cm. per cm. per degree C. In particular, I have found particularly good seals to be produced between boro-silicate glasses having expansivities between 3.0 and  $5.5 \times 10^{-6}$  cm. per cm. per degree C. and alloys containing substantially 50 29.8% nickel, 15.5% cobalt, 0.22% manganese and 0.3% carbon. Boro-silicate glasses having expansivities of substantially  $3.6 \times 10^{-6}$  cm. per cm. per degree C. apparently produce the best seals with the alloy last mentioned.

I have also found that a seal between the boro-silicate glass known to the trade as G702P and manufactured by the Corning Glass Company, seals well with a lead comprising 29.4% 60 nickel, 16.3% cobalt, 0.2% manganese and the remainder iron. I have also obtained excellent seals between the same glass and a lead coated with chromium or copper and consisting of an alloy containing substantially 23.8% nickel, 21.9% cobalt, 0.2% manganese, 0.3% carbon and the remainder iron.

In general, I have found that, in the case of alloys of low expansivity containing nickel and iron, whether or not they also contain cobalt, 65 it is desirable that the relationship expressed by the following formula should hold:

$$\frac{\% \text{ nickel} + 2.5 (\% \text{ manganese}) + 18 (\% \text{ carbon})}{\% \text{ iron}} = 0.60 \text{ to } 0.80$$

70 the best value for the fraction being about 0.55.

It also appears desirable, for most purposes, to minimize the amount of manganese, the maximum percentage of this element being preferably below 0.2%. Carbon, however, appears, in most instances, to be desirable up to the amount 5 of 0.3%, as it prevents a higher cobalt content than would otherwise be desirable and does not seriously affect expansivity.

As previously stated, I have found certain 10 nickel-cobalt-iron alloys to seal successfully into ordinary lead glass having a coefficient of expansion in the neighborhood of  $9 \times 10^{-6}$  cm. per cm. per degree C. For instance, alloys comprising 15 30% to 45% nickel, 5% to 25% cobalt and 0 to 1% manganese, form satisfactory seals with lead glass having an expansivity between  $6 \times 10^{-6}$  and  $10 \times 10^{-6}$  cm. per cm. per degree C.

I have found that the preparation of vacuum-tight seals between metals and glass is rendered more certain if the metals are annealed in vacuo 20 or in a bath of a fused salt which readily dissolves the oxides of the metal. For example, sodium nitrate is one such salt, many others being known to skilled chemists.

I have also found that a certain amount of 25 trouble is caused in making vacuum-tight seals because of gases released at a high temperature, and largely results from a reaction between carbon in the metal and oxide formed on the surface 30 of the metal during heating in air.

This source of gas may be eliminated either by removing carbon from the metal or by coating the metal with another metal which is impervious to oxygen and contains no carbon.

Small amounts of carbon cannot be avoided in 35 iron-base alloys without elaborate precautions. Consequently, it is more convenient to remove the carbon from the alloy than to prevent its introduction therein. Carbon may be removed from the molten alloy by maintaining it in a vacuum 40 in contact with refractory oxides or by passing hydrogen through the metal. This treatment is preferable when the finished piece is bulky. When, however, the metal is finished to a small cross-section, the carbon may be removed conveniently from the solid metal. The treatment required is heating at an appropriate temperature 45 in hydrogen or in a fused salt bath containing no great amount of carbon compounds. A bath comprising 15% sodium chloride and 85% barium 50 chloride at from 700° to 1200° centigrade is one suitable bath.

Coating to avoid gas generation at the surface 55 may be readily accomplished by electrolytic deposition of a thin layer of chromium or other carbon-free metal provided that the oxygen-carbon relations within the alloy are not such as to cause severe gas release at working temperatures. In the event that gas is evolved without surface oxidation, a treatment, such as that just described, 60 may first be applied to prevent injury to the coating by the gas. This treatment is particularly applicable to plated metals intended for high-temperature service.

The temperature at which strains are readily 65 relieved in glass is, of course, not an absolutely fixed quantity, even for glass of a given chemical composition. At very high temperatures, the glass is relatively soft and, as the temperature decreases, it hardens. The lower the temperature 70 and, consequently, the harder the glass, the less rapidly it is able to flex and relieve mechanical strains existing within it. However, since the inflection temperature, that is to say, the maximum temperature, at which coefficient of expansion 75

sion of the above-described alloys remain low, decreases as the coefficient of expansion itself is decreased, it is desirable to form seals with as low an annealing temperature as possible. I have found that alloys, in which the inflection temperature is relatively low, may be employed to produce satisfactory seals if the completed seal is maintained at a temperature of about 50° C. above the inflection temperature for a considerable period of time. Thus, while the strains are relieved slowly, they do so progressively and with certainty, and a strong vacuum-tight seal results in the end.

As an example of the softer glasses, referred to above as lead glasses, the following may be taken as typical in composition:

63.1%  $\text{SiO}_2$ ; 20.2%  $\text{PbO}$ ; 0.28%  $\text{Al}_2\text{O}_3$ ; 0.94%  $\text{CaO}$ ; 7.6%  $\text{NaO}$ ; 5.5%  $\text{K}_2\text{O}$ ; 0.88%  $\text{Mn}_3\text{O}_4$

The above subject matter is also described and referred to in my copending application Serial No. 376,292, filed July 5, 1929, for Alloys, now Patent No. 1,942,260, issued January 2, 1934.

While I have, in the foregoing, described certain particular embodiments of my invention, it will be understood that these are for purposes of illustration only, and that the broad principles may be otherwise utilized, as will be readily apparent to those skilled in the art. I, accordingly, desire that the following claims shall be accorded the broadest construction of which their terms are susceptible in view of the limitations imposed by the prior art.

I claim as my invention:

1. A vacuum tight seal between an alloy comprising 28% to 34% nickel, 5% to 25% cobalt, less than 1% manganese and the remainder iron, and a boro-silicate glass.

2. A vacuum tight seal between an alloy comprising 24% to 34% nickel, 5% to 25% cobalt, less than 1% manganese and the remainder iron, and a boro-silicate glass having an expansivity of 3.0 to  $6.5 \times 10^{-6}$  centimeters per centimeter per degree centigrade.

3. A vacuum tight seal between an alloy comprising 24% to 34% nickel, 5% to 25% cobalt, less than 1% manganese and the remainder iron, and a glass having a composition of 73.8%  $\text{SiO}_2$ ; 18.7%  $\text{B}_2\text{O}_3$ ; 5.2%  $\text{PbO}$ ; 1.0%  $\text{Al}_2\text{O}_3$ ; 0.5%  $\text{As}_2\text{O}_3$ .

4. A vacuum tight seal between boro-silicate glass and an alloy having essentially iron, nickel and cobalt.

5. A vacuum tight seal between glass having an expansivity of 3.0 to  $6.5 \times 10^{-6}$  centimeters per centimeter per degree centigrade and an alloy having essentially iron, nickel and cobalt.

6. A vacuum tight seal between a glass containing substantially 73.8%  $\text{SiO}_2$ ; 0.5%  $\text{As}_2\text{O}_3$ ; 5.2%  $\text{PbO}$ ; 1.0%  $\text{Al}_2\text{O}_3$ ; 18.7%  $\text{B}_2\text{O}_3$  and an iron-base alloy containing substantially 29.8% nickel,

15.5% cobalt, 0.22% manganese and less than 0.1% carbon.

7. A vacuum tight seal between a boro-silicate glass and an alloy containing chiefly iron, nickel, cobalt, manganese and carbon in such proportions that the present nickel content plus 2.5 times the percent manganese content plus 18 times the percent carbon content divided by the percent iron content is between 0.50 and 0.60.

8. A vacuum tight seal between a conductor comprising an alloy containing substantially 24 to 34% nickel, 10 to 25% cobalt, less than 1% manganese and the remainder iron and a boro-silicate glass containing 65 to 75%  $\text{SiO}_2$ , less than 10%  $\text{PbO}$ , less than 6%  $\text{Al}_2\text{O}_3$  and 10 to 25%  $\text{B}_2\text{O}_3$ .

9. A vacuum tight seal between a conductor comprising an iron-base alloy containing substantially 29.8% nickel, 15.5% cobalt, 0.22% manganese less than 0.1% carbon and the remainder iron and a boro-silicate glass having an expansivity of 3.0 to  $5.5 \times 10^{-6}$  centimeters per centimeter per degree centigrade.

10. An electrical discharge device comprising at least two electrodes, insulation between said electrodes comprising glass having an expansivity of 3.0 to  $6.5 \times 10^{-6}$  centimeters per centimeter per degree centigrade and an alloy having essentially iron, nickel and cobalt sealed vacuum-tight through said glass.

11. An electrical discharge device comprising at least two electrodes, insulation between said electrodes comprising boro-silicate glass and an alloy having essentially iron, nickel and cobalt sealed through said glass.

12. An electrical discharge device comprising at least two electrodes, insulation between said electrodes comprising boro-silicate glass and an alloy comprising 24 to 34% nickel, 5% to 25% cobalt, less than 1% manganese and the remainder iron, sealed vacuum-tight through said glass.

13. An electrical discharge device comprising a container having a wall portion comprising glass having an expansivity of 3.0 to  $6.5 \times 10^{-6}$  centimeters per centimeter per degree centigrade, and an alloy comprising 24 to 34% nickel, 5% to 25% cobalt, less than 1% manganese and the remainder iron, sealed vacuum tight through said glass.

14. An electrical discharge device comprising a container having a wall portion comprising boro-silicate glass and an alloy comprising 24 to 34% nickel, 5% to 25% cobalt, less than 1% manganese and the remainder iron, sealed vacuum tight through said glass, said glass containing 65% to 75%  $\text{SiO}_2$ , less than 10%  $\text{PbO}$ , less than 6%  $\text{Al}_2\text{O}_3$  and 10 to 25%  $\text{B}_2\text{O}_3$ .

HOWARD SCOTT.